

1

3,466,171

## NICKEL-CHROMIUM-NIOBIUM ALLOY

Alfred John Fletcher, Birmingham, and Edward Gordon Richards, Worcestershire, England, assignors to The International Nickel Company, New York, N.Y., a corporation of Delaware

No Drawing. Filed July 18, 1966, Ser. No. 565,711  
Claims priority, application Great Britain, July 20, 1965,

30,785/65

Int. Cl. C22c 19/00; C22f 1/11

U.S. Cl. 75—171

10 Claims

### ABSTRACT OF THE DISCLOSURE

Nickel-chromium alloys containing niobium, substantial amounts of carbon and, advantageously, molybdenum, wherein the niobium, carbon, chromium and molybdenum constituents of the alloys are carefully correlated to obtain good stress-rupture properties at 900° C. and higher.

This invention relates to nickel-base alloys capable of sustaining high stress at elevated temperatures for prolonged periods before fracture occurs and, more particularly, to nickel-chromium alloys, containing both niobium and carbon, which display these high strength properties.

Most prior art nickel-base alloys depend for their high-temperature strength upon the formation of precipitates of phases containing nickel and also titanium or aluminum or both, commonly referred to as the gamma prime phase ('gamma') represented by the formula  $Ni_3(Ti, Al)$ . Other prior art alloys contain niobium and are strengthened, though less effectively, by a precipitated nickel niobide phase, and in yet others, phases of both kinds are present. In most of these alloys, however, the carbon content is kept low, below 0.2% or even less, in order to minimize the formation of carbides of the addition elements at the expense of the desired intermetallic phases. Such carbides are undesirable because in the temperature range in which the intermetallic phases are effective to harden and strengthen the alloys, carbides are less effective for this purpose.

As the temperature increases, the stress-rupture life of the alloys of the types above described decreases. This is due mainly to the instability of the intermetallic phase which tends to coarsen at elevated temperatures, thereby becoming less effective to strengthen the alloys, and eventually to dissolve and, to a lesser extent, to loss of strength by the matrix. At temperatures above 900° C., the stress-rupture life of even the strongest alloys hardened by intermetallic phases falls off rapidly.

A further disadvantage of alloys containing titanium and aluminum is that upon cooling from hot-working temperatures the alloys harden very rapidly. Hence, when the alloys are to be used in the form of sheet they must be quenched after hot working in order that the sheet may be soft enough to be conveniently fabricated by cold forming. It is very difficult to quench the sheet material successfully without distortion occurring, especially in large pieces. Moreover, the strongest alloys, i.e., those with the highest titanium and aluminum contents, cannot be used in the form of sheet since the rate of hardening increases with increasing titanium and aluminum contents and such alloys cannot be sufficiently softened even by very rapid quenching.

The present invention is based on the discovery that these problems can be largely overcome by the use of niobium and carbon, within clearly defined limits, as hardening additions to nickel-chromium alloys of special composition.

2

It is an object of this invention to provide nickel-base alloys which maintain high strength at temperatures of 900° C. and above.

Another object of this invention is to provide nickel-base alloys which, when compared with nickel-base alloys hardened by precipitation of the gamma prime phase, do not appreciably harden on cooling from high temperatures.

Generally speaking, the present invention contemplates alloys comprising (percent by weight) about 2% to about 6% niobium, about 0.3% to about 0.5% carbon, about 19% to about 33% chromium, an amount of molybdenum such that:

(i) When the chromium content is less than 24% the molybdenum content is at least that given by the expression

$$\text{percent Mo} = \frac{1}{2} (24 - \text{percent Cr})$$

(ii) When the chromium content does not exceed 30% the molybdenum content is from 0 to that given by the expression

$$\text{percent Mo} = 3.5 + 0.5 (30 - \text{percent Cr})$$

and  
(iii) When the chromium content is greater than 30% the molybdenum content is from 0 to about 3.5%, up to about 0.01% boron, up to about 0.1% zirconium, up to about 3% iron, up to about 2% cobalt, up to about 2% silicon, up to about 1% manganese, and the balance being essentially nickel with residual impurities and deoxidants, e.g., magnesium and/or calcium, in ordinary amounts which do not affect the basic characteristics of the alloys.

In accordance herewith we have found that niobium contributes importantly to the stress-rupture strength of the alloys. For adequate stress-rupture life at least 2.0% niobium is required, while preferably at least 2.5% is present and most advantageously at least 3.5%. Increasing the niobium content above the maximum of 6%, however, leads to a rapid drop in stress-rupture strength, and the impact strength of the alloys also decreases somewhat as the niobium content increases.

Carbon is of great importance in the alloys, since it plays a large part in controlling the hardening and strengthening mechanisms. As the carbon content is increased above 0.2%, the stress-rupture life rapidly increases, but at the same time the impact strength decreases and at carbon contents above 0.5% it becomes inadequate.

To obtain the benefit of the strengthening effects of niobium and carbon, the contents of chromium and molybdenum must be correlated. Chromium contributes to the stress-rupture strength of the alloys, and in the absence of molybdenum the alloys must contain at least 24% chromium. Chromium also contributes to corrosion resistance, and if the highest corrosion resistance is required the chromium content should be high, i.e., at least 28%. On the other hand with increasing chromium contents the impact strength decreases and if the highest impact strength is important, the chromium content should not exceed 25%. Alloys with high chromium contents are also difficult to work, and if the chromium content exceeds 33% they are unforgeable.

We have surprisingly found that although molybdenum does not improve the stress-rupture strength of alloys that are free from niobium, it is very effective in the niobium-containing alloys of the invention. When the chromium content is less than 24% it must be present, and at all chromium contents at least 1% molybdenum is preferred. The effects of chromium and molybdenum are complementary, and as the chromium content increases the amount of molybdenum needed to achieve a given stress-rupture strength decreases. Excessive amounts of molybdenum cause the stress-rupture strength to fall again, and the maximum amount that may be present decreases

with increasing chromium content in accordance with the formula

$$\text{percent Mo} = 3.5 + 0.5 \text{ (30-percent Cr)}$$

until at chromium contents of 30% and above the molybdenum content must not exceed 3.5%. The optimum stress-rupture properties are obtained when the chromium and molybdenum contents are correlated in accordance with the formula

$$\text{percent Mo} = 3.5 + 0.4 \text{ (30-percent Cr)}$$

In contrast to alloys strengthened by intermetallic phases containing titanium and aluminum, the stress-rupture properties of the alloys of the invention are not improved by additions of boron or zirconium. If desired, however, these elements may be present in amounts up to 0.01% boron or 0.1% zirconium or both, e.g., 0.005% boron and 0.03% zirconium. Nevertheless such additions impair the weldability of the alloys, so boron and zirconium are preferably not added in making sheet and other forms where good weldability is important.

As to the other constituents, iron and cobalt impair the stress-rupture lives of the alloys. For this reason the amount thereof should not exceed 3% iron and 2% cobalt respectively and advantageously should not be above impurity levels. Preferably both are substantially absent. Silicon impairs weldability and if good weldability is required the silicon content should not exceed 0.3%. If weldability is not of importance, the silicon content may be as high as 0.5% or even 1% or 2%. Up to 1% manganese may be present as an impurity.

To facilitate hot working the alloys it is desirable that they should contain small residual amounts of magnesium or calcium, e.g., up to 0.035%. Such amounts are commonly present after the use thereof as deoxidants in air melting and if vacuum-melting is employed it is also advantageous to add them before casting the alloy.

An advantageous combination of results is obtained when the alloys contain about 24% to about 33% chromium, about 0.3% to about 0.5% carbon, about 2% to about 6% niobium, about 1% to about 3.5% molybdenum, up to about 0.005% boron, up to about 0.03% zirconium, up to about 0.3% silicon, up to about 1% manganese, up to about 0.035% magnesium, up to about 0.035% calcium, and the balance essentially nickel. A particularly advantageous alloy has the composition 30% chromium, 5% niobium, 2.5% molybdenum, 0.4% carbon and the balance essentially nickel.

The hardening phases that form in the alloys of our invention remain largely undissolved at temperatures at which the gamma' phase dissolves in prior art nickel-chromium alloys hardened by titanium and aluminum. Moreover, the hardening phases of our alloys are not completely dissolved even at temperatures only slightly below the melting-point of the alloys. Thus, the alloys in

Despite the relative insolubility of the hardening phases at high temperatures, enough can be dissolved for substantial further precipitation to occur on subsequent aging at a lower temperature and, in order to develop the stress-rupture properties to the fullest extent, the alloys require 5 heat treatment by solution-heating and aging. The higher the temperature of solution heating, the better the stress-rupture properties after aging. Advantageously the solution heating temperature is at least 1125° C., e.g., 1150° C. or even 1250° C., but it should not be so high that incipient melting occurs. A suitable period of heating is from one-half to eight hours, though longer periods may be used if desired.

The alloys may be cooled from the solution-heating 10 temperature at any convenient rate either directly to the aging temperature or to a lower temperature, conveniently room temperature, followed by reheating to the aging temperature. The rate of cooling from the solution-heating temperature has little effect upon the hardness, and 15 even after air-cooling to room temperature, the hardness of the alloys in the form, for example, of  $\frac{5}{8}$  inch diameter bar or sheet, is generally low enough to permit heavy machining of the bar stock and cold-forming of the sheet. However if the highest stress-rupture strength is 20 required it is advantageous to cool the alloys rapidly from the solution-heating temperature, e.g., by water-quenching. Aging is suitably performed in the range of 750° C. to 1060° C., e.g., at 850° C., for about 1 to 48 hours. The duration of aging depends on the temperature, and 25 at 850° C. is conveniently 16 hours.

For the purpose of giving those skilled in the art a better understanding of the invention, the results of numerous tests carried out on alloys of different compositions both within and without the invention are reproduced in several 30 tables shown below. As is reflected by these results, the good stress-rupture properties of the alloys of this invention depend on a delicate balance among the alloying elements. The alloys used were prepared by air-melting with a conventional addition of magnesium or calcium as 35 a deoxidant, casting to ingots, forging to  $\frac{5}{8}$  inch diameter bars, solution-heating for 2 hours at 1150° C., air-cooling, and finally aging for 16 hours at 850° C. Suitable test samples were thereafter machined from the aged bars. Stress-rupture properties were determined at 900° C., and 40 45 Charpy impact strengths were determined at room temperature after soaking for 1,000 hours at 850° C. to reveal any tendency of the alloys to embrittle in service.

Table I contains stress-rupture and impact data for 50 alloys containing varying amounts of niobium and molybdenum with each alloy nominally containing 30% chromium and 0.4% carbon, the balance being nickel. Alloys Nos. 1 to 4 are alloys according to the invention whereas Alloy A, which contained no niobium, and alloys B and C, which nominally contained 7% niobium, are not.

TABLE I

| Alloy No. | Nb<br>(percent) | Mo<br>(percent) | Stress-rupture properties |                     |                  |                     | Impact<br>strength<br>(ft.-lb.) |
|-----------|-----------------|-----------------|---------------------------|---------------------|------------------|---------------------|---------------------------------|
|           |                 |                 | 3 t.s.i./900° C.          |                     | 2 t.s.i./900° C. |                     |                                 |
|           |                 |                 | Life<br>(hr.)             | Elong.<br>(percent) | Life<br>(hr.)    | Elong.<br>(percent) |                                 |
| A-----    | 0               | 0               | -----                     | -----               | 167              | -----               | -----                           |
| 1-----    | 3               | 0               | 151                       | 18                  | 687              | -----               | 24                              |
| 2-----    | 5               | 0               | 492                       | 23                  | 2,063            | 26                  | 11                              |
| B-----    | 7               | 0               | 98                        | 51                  | -----            | -----               | -----                           |
| 3-----    | 2.5             | 2.5             | -----                     | -----               | 2,145            | 30                  | 20                              |
| 4-----    | 5               | 2.5             | 654                       | 27                  | >1,063           | >0.7                | 6                               |
| C-----    | 7               | 2.5             | 86                        | 23                  | -----            | -----               | -----                           |

<sup>1</sup> Test discontinued because of very low creep rate.  
t.s.i.=long tons/in.<sup>2</sup>.

accordance herewith retain high strength at temperatures of 900° C. and above. In addition, the alloys do not harden as rapidly and as extensively on cooling from high temperature as do the alloys hardened by gamma' phase.

Alloys A and B, in which the niobium contents were 75 respectively lower and higher than are required by the invention, had much inferior stress-rupture lives in comparison with Alloys Nos. 1 and 2, and Alloy C was likewise much inferior to Alloys Nos. 3 and 4. Comparison of

Alloy No. 2 with Alloy No. 1 and of Alloy No. 4 with Alloy No. 3 also illustrates the concurrent increase in stress-rupture life and decrease in impact strength that results from increasing the niobium content.

The role of carbon is shown by the results reported in Table II relating to alloys containing 30% chromium with varying amounts of carbon, niobium and molybdenum, the balance being nickel. Alloys Nos. 1, 2, 3 and 4, being examples of the invention, are reproduced for purposes of the comparison with Alloys D, E, F, G and H which are not examples of this invention since the carbon content is either too low or too high.

It is essential that the alloy contains both niobium and carbon in order to form strengthening phases rich in niobium.

Although no reliance is placed upon any particular theory to explain the invention, it is believed that the good stress-rupture properties possessed by the alloys of our invention at temperatures of 900° C. and above are due to the presence in dispersed form of niobium carbide NbC, with or without the nickel niobide Ni<sub>3</sub>Nb. The phase Cr<sub>23</sub>C<sub>6</sub> is frequently present and may also cooperate with the niobium-rich phases to strengthen the alloys, though it is not very effective alone at high temperatures.

TABLE II

| Alloy No. | C<br>(percent) | Nb<br>(percent) | Mo<br>(percent) | Stress-rupture properties |                     |                              |                     |
|-----------|----------------|-----------------|-----------------|---------------------------|---------------------|------------------------------|---------------------|
|           |                |                 |                 | 3 t.s.i./900° C.          | 2 t.s.i./900° C.    | Impact strength<br>(ft.-lb.) |                     |
|           |                |                 |                 | Life<br>(hr.)             | Elong.<br>(percent) | Life<br>(hr.)                | Elong.<br>(percent) |
| D         | 0.2            | 2.9             | 0               | 95                        | 32                  | -----                        | 34                  |
| 1         | 0.4            | 3.0             | 0               | 151                       | 18                  | 687                          | 24                  |
| E         | 0.2            | 5.1             | 0               | 131                       | 31                  | -----                        | 14                  |
| 2         | 0.4            | 5               | 0               | 492                       | 23                  | 2,063                        | 14                  |
| F         | 0.6            | 5               | 0               | 95                        | 41                  | 26                           | 11                  |
| G         | 0.2            | 3.0             | 2.7             | -----                     | 61                  | 48                           | 37                  |
| 3         | 0.4            | 2.5             | 2.5             | -----                     | 2,145               | 30                           | 20                  |
| H         | 0.2            | 5.1             | 2.8             | 92                        | 26                  | -----                        | 6                   |
| 4         | 0.4            | 5               | 2.5             | 654                       | 27                  | -----                        | -----               |

Irrespective of the niobium and molybdenum contents, in every instance the alloys with 0.2% carbon (Alloys D, E, G and H) and with 0.6% carbon (Alloy F) were substantially inferior to otherwise comparable alloys containing 0.4% carbon.

The effects on stress-rupture and impact properties of varying the chromium and molybdenum contents are illustrated by the results in Table III, which all relate to alloys containing 0.4% carbon. Comparison of Alloys A and J

30 The importance of the presence of niobium-rich phases is shown by the results in Table IV, in which niobium-free Alloys A, M, N and J are hardened by Cr<sub>23</sub>C<sub>6</sub> alone and have relative poor stress-rupture lives and are, therefore, not within the scope of this invention. In contrast, Alloy 35 No. 2 contains 5% niobium and is strengthened by the precipitation of the niobide phases, NbC and Ni<sub>3</sub>Nb, and is, therefore, an alloy within the teachings of this invention.

TABLE IV

| Alloy No. | Nb<br>(percent) | Mo<br>(percent) | W<br>(percent) | Stress-rupture properties, 2 t.s.i./900° C. |                     |                                                            |
|-----------|-----------------|-----------------|----------------|---------------------------------------------|---------------------|------------------------------------------------------------|
|           |                 |                 |                | Life<br>(hr.)                               | Elong.<br>(percent) | Phases present                                             |
| 2         | 5               | 0               | 0              | 2,063                                       | 26                  | NbC, Ni <sub>3</sub> Nb<br>Cr <sub>23</sub> C <sub>6</sub> |
| A         | 0               | 0               | 0              | 167                                         | -----               | Cr <sub>23</sub> C <sub>6</sub>                            |
| M         | 0               | 0               | 5.0            | 187                                         | 38                  | Cr <sub>23</sub> C <sub>6</sub>                            |
| N         | 0               | 2.5             | 2.5            | 479                                         | 10                  | Cr <sub>23</sub> C <sub>6</sub>                            |
| J         | 0               | 4.9             | 0              | 118                                         | 24                  | Cr <sub>23</sub> C <sub>6</sub>                            |

(neither of which is in accordance with the invention) shows the ineffectiveness of a molybdenum addition in the absence of niobium. The series of Alloys 2, 4 and K and the series Nos. L, 6, 7 and 8 show the effects of increasing the molybdenum content at chromium contents of 30% and 20% respectively: all these alloys are examples of the invention except Alloy K, which contains too much molybdenum with 30% chromium, and Alloy L, which contains only 20% chromium and no molybdenum. Each of these had poor stress-rupture properties. The effect of varying chromium alone is shown by comparison of 60 Alloys 2, 5 and L.

50 It is worthy of mention that tungsten is not equivalent to molybdenum in the alloys and in addition is never beneficial and frequently detrimental to both the stress-rupture life and the impact strength. This is shown by Table V in which Alloy Nos. 2 and 4 are compared with Alloy P, an alloy nominally identical with Alloy No. 2 except for the inclusion of 2.6% tungsten. It will be seen that the life to rupture and impact strength is considerably reduced by the tungsten. Moreover, Alloy No. 4, which contains 2.5% molybdenum, shows a considerable increase in stress-rupture life over Alloy No. 2 and Alloy K. Accordingly, the alloys of this invention do not require tungsten as a constituent thereof and are preferably tungsten-free.

TABLE III

| Alloy No. | Cr<br>(percent) | Nb<br>(percent) | Mo<br>(percent) | Stress-rupture properties |                     |                              |                     |
|-----------|-----------------|-----------------|-----------------|---------------------------|---------------------|------------------------------|---------------------|
|           |                 |                 |                 | 3 t.s.i./900° C.          | 2 t.s.i./900° C.    | Impact strength<br>(ft.-lb.) |                     |
|           |                 |                 |                 | Life<br>(hr.)             | Elong.<br>(percent) | Life<br>(hr.)                | Elong.<br>(percent) |
| A         | 30              | 0               | 0               | -----                     | 167                 | -----                        | -----               |
| J         | 30              | 0               | 4.9             | -----                     | 118                 | 24                           | 19                  |
| 2         | 30              | 5               | 0               | 492                       | 22                  | 2,063                        | 26                  |
| 4         | 30              | 5               | 2.5             | 654                       | 27                  | -----                        | 11                  |
| K         | 30              | 5               | 5               | 105                       | -----               | -----                        | -----               |
| 5         | 25              | 5               | 0               | 431                       | 38                  | -----                        | 30                  |
| L         | 20              | 5               | 0               | 103                       | 41                  | -----                        | 56                  |
| 6         | 20              | 5               | 2.5             | -----                     | -----               | -----                        | 46                  |
| 7         | 20              | 5               | 5               | 675                       | 30                  | -----                        | 29                  |
| 8         | 20              | 5               | 7.5             | 743                       | 26                  | -----                        | 15                  |

TABLE V

| Alloy No. | Nb<br>(percent) | Mo<br>(percent) | W<br>(percent) | Stress-rupture proper-<br>ties, 3 t.s.i./900° C. |                     |                                 |
|-----------|-----------------|-----------------|----------------|--------------------------------------------------|---------------------|---------------------------------|
|           |                 |                 |                | Life<br>(hr.)                                    | Elong.<br>(percent) | Impact<br>strength<br>(ft.-lb.) |
| 2-----    | 5-----          | -----           | 0              | 492                                              | 23                  | 11                              |
| P-----    | 5.1-----        | -----           | 2.6            | 50                                               | 40                  | 6                               |
| 4-----    | 5-----          | 2.5-----        | -----          | 654                                              | 27                  | 6                               |

We have also found that tantalum is not equivalent to niobium in the alloys, and replacement of part of the niobium by an equiatomic amount of tantalum drastically reduces the stress-rupture strength. This is shown by the results in Table VI, in which Alloy No. 4 is compared with an alloy (Alloy Q) nominally identical except for the replacement of 2.5% niobium by 5% tantalum.

TABLE VI

| Alloy No. | Nb<br>(percent) | Ta<br>(percent) | Mo<br>(percent) | Stress-rupture proper-<br>ties, 3 t.s.i./900° C. |                     |
|-----------|-----------------|-----------------|-----------------|--------------------------------------------------|---------------------|
|           |                 |                 |                 | Life (hr.)                                       | Elong.<br>(percent) |
| 4-----    | 5-----          | -----           | 2.5             | 654                                              | 27                  |
| Q-----    | 2.5             | 5               | 2.5             | 78                                               | 34                  |

Tantalum should therefore not be added to the alloys, though it may be tolerated as an impurity in the amounts commonly found as an impurity in commercial sources of niobium, i.e. in amounts up to about one-tenth of the weight of niobium.

The good corrosion-resistance of an alloy according to the invention is shown by the results of a test in which a specimen of Alloy No. 2 was half-immersed for 16 hours in a molten bath of a mixture of 25% sodium chloride and 75% sodium sulphate at 900° C. The loss in weight of the specimen was only 14 mg./cm.<sup>2</sup>.

The advantageous properties of the alloys of the invention make them suitable for use at elevated temperatures which may exceed 900° C., in the form of sheet and components fabricated therefrom. They are also useful for articles and parts that require a combination of strength and resistance to corrosion at such temperatures, for example as parts of heat-treatment furnaces, furnace belts, e.g., wire mesh belts, trays for articles to be heat-treated, and the like.

We claim:

1. An alloy, age-hardenable by precipitation of at least one niobium-rich phase, and consisting essentially of about 2% to about 6% niobium, about 0.3% to about 0.5% carbon, about 19% to about 33% chromium, and amount of molybdenum such that when the chromium content is less than 24% the molybdenum content is at least 5% (24-percent Cr) percent; when the chromium content

10 does not exceed 30% the molybdenum content is from 0 to 3.5+0.5 (30-percent Cr) percent; and when the chromium content is greater than 30% the molybdenum content is from 0 to 3.5%, up to about 0.01% boron, up to about 0.1% zirconium, up to about 3% iron, up to about 15 about 2% cobalt, up to about 2% silicon, up to about 1% manganese, and the balance essentially nickel.

2. The alloy set forth in claim 1 and containing at least 2.5% niobium.

3. The alloy set forth in claim 2 and containing at least 20 about 1% molybdenum.

4. The alloy set forth in claim 3 in which boron does not exceed about 0.005% and zirconium does not exceed 0.03%.

5. The alloy set forth in claim 4 in which silicon does 25 not exceed 1%.

6. The alloy recited in claim 1 and containing about 24% to about 33% chromium, about 2% to about 6% niobium, about 1% to about 3.5% molybdenum and about 0.3% to about 0.5% carbon.

30 7. The alloy set forth in claim 6 in which the chromium content is at least 28%.

8. The alloy set forth in claim 7 in which silicon does not exceed 1%.

9. The alloy set forth in claim 6 in which the niobium 35 content is at least about 3.5%.

10. The alloy set forth in claim 6 and containing about 30% chromium, about 5% niobium, about 0.4% carbon, about 2.5% molybdenum and the balance essentially nickel.

40

#### References Cited

#### UNITED STATES PATENTS

|              |         |             |       |        |
|--------------|---------|-------------|-------|--------|
| 2,587,275    | 2/1952  | Bash        | ----- | 75—171 |
| 45 2,994,605 | 8/1961  | Gill et al. | ----- | 75—171 |
| 3,046,108    | 1/1962  | Eiselstein  | ----- | 75—171 |
| 3,069,258    | 12/1962 | Haynes      | ----- | 75—171 |
| 3,046,108    | 7/1962  | Eiselstein  | ----- | 75—171 |

50 RICHARD O. DEAN, Primary Examiner

U.S. Cl. X.R.

148—162

UNITED STATES PATENT OFFICE  
CERTIFICATE OF CORRECTION

Patent No. 3,466,171 Dated September 9, 1969

Inventor(s) Alfred John Fletcher and Edward Gordon Richards

It is certified that error appears in the above-identified patent and that said Letters Patent are hereby corrected as shown below:

Column 5, line 60, delete entire line reading  
"wise much inferior to Alloys Nos. 3 and 4. Comparison of"  
Column 6, line 32, for "relative", read --relatively--.  
Column 6, line 57, for "contain", read --contains--.  
Column 7, line 50, for "and", read --an--.

SIGNED AND  
SEALED  
NOV 17 1970

(SEAL)

Attest:

Edward M. Fletcher, Jr.

Attesting Officer

WILLIAM H. SCHUYLER, JR.  
Commissioner of Patents